

# UNITED STATES PATENT OFFICE.

JOSEPH CHARLES MORRIS, OF FINDLAY, OHIO.

## METALLURGICAL PROCESS.

979,541.

Specification of Letters Patent. Patented Dec. 27, 1910.

No Drawing.

Application filed September 6, 1910. Serial No. 580,513.

*To all whom it may concern:*

Be it known that I, JOSEPH CHARLES MORRIS, a citizen of the United States of America, residing at Findlay, in the county of 5 Hancock and State of Ohio, have invented a new and useful Metallurgical Process, of which the following is a specification, to wit:

This invention relates to a process for the 10 production of a metallic compound peculiarly adapted for the making of tools, parts of machines and other articles, by casting, rather than by forging or rolling or otherwise working the metal as has heretofore been commonly done.

One of the principal objects of the invention is the production of a metal possessing great hardness and toughness without tempering, while at the same time being capable of having its hardness increased by 20 tempering if desired, the untempered product, however, being capable of retaining a cutting edge when used for tools or other articles if desired.

25 It will be readily apparent, to those skilled in the art, that other valuable results are obtained through my invented process, the product of such process being adapted for many purposes and uses other than those 30 above mentioned.

In the carrying out of my process, I first place in a crucible or melting pot, fifty pounds of broken iron castings, or any ordinary iron such as "common cast iron" being suitable. I then add fifty pounds of 35 steel clippings or borings such as are ordinarily produced in machine shops, applying sufficient heat to melt said iron and clippings. When the iron and steel are at the 40 point of fusing I add, preferably at the same time, one ounce of aluminum (Al.) one ounce of magnesium (Mg.) and one pound of silica ( $SiO_2$ ). After thoroughly fusing together the iron, steel, aluminum, 45 magnesium and silica the compound should be poured into suitable molds for the making of the tool or other casting desired. The casting, when cool is removed from the mold when it may be dressed in all the usual ways, 50 on an emery wheel or otherwise and in the

case of a tool, an edge may be ground upon the same. Without tempering, the tools, thus formed, will be found to retain an edge in an admirable manner, even in the case of cold chisels, and the like which are frequently subjected to very severe and rough usage. If it is desired to further harden the casting, it may be heated and tempered in the same manner as is customarily employed in the tempering of steel. 55

Attention should be called to the fact that by my process it is possible to produce a desirable metallic compound suitable for the most exacting requirements at a cost below the cost of the same articles made from steel 60 in the usual way, while the compound produced requires no further tempering except for unusually severe usage.

I claim:

1. That metallurgical process which consists in compounding and fusing iron, steel, aluminum, magnesium and silica, as and for the purpose specified. 70

2. That metallurgical process which consists in fusing iron and steel in a suitable 75 container, adding aluminum, magnesium and silica while said iron and steel are in a fused condition and casting the compound thus formed in a mold.

3. That metallurgical process which consists in fusing equal parts, by weight, of iron and steel, adding a quantity of aluminum, magnesium and silica, and pouring the compound, while in a fused condition, into molds. 80

4. That metallurgical process which consists in fusing fifty pounds of broken iron castings or "common cast iron" and fifty pounds of steel clippings and, when at the point of fusing, adding one ounce of aluminum, one ounce of magnesium and one pound 90 of silica, and casting the same in a mold.

In testimony that I claim the above, I have hereunto subscribed my name in the presence of two witnesses.

JOSEPH CHARLES MORRIS.

Witnesses:

JOSEPH KOCH,  
N. H. REILLY.